

## UNITED STATES PATENT OFFICE

VINCENT M. VERTUCCI, OF JERSEY CITY, NEW JERSEY

## METHOD OF PREPARING CHROMIUM-PLATED FERROUS ARTICLES

No Drawing.

Application filed October 7, 1926. Serial No. 140,219.

The desirable characteristics of electrical-  
ly deposited chromium metal are well  
known. The chromium coating is extremely  
hard and resists abrasion very well; it has  
5 a pleasing blue-white color and is capable  
of taking and retaining a high polish; it  
resists the corrosive action of the atmos-  
phere, sea-water, and many acids, including  
the common food acids; and it resists oxi-  
10 dation even at high temperatures. This  
combination of desirable properties renders  
it particularly suitable for coating a great  
variety of commercial products, and more  
particularly articles of iron or steel.

15 Thin, adherent coatings of chromium can  
readily be deposited upon clean surfaces of  
iron or steel; but investigation has shown  
that these coatings as heretofore prepared,  
are not continuous over considerable areas,  
20 but present defects of the nature of minute  
unplated areas, or so-called pin holes, where  
the underlying metal is subject to attack.  
This difficulty has been partially overcome  
in the past by preliminarily coating the  
25 iron or steel with copper or nickel, which  
may increase the total protective effect, even  
though it does not very greatly improve the  
continuity of the chromium film.

I have made the surprising discovery that  
30 continuous or practically continuous films of  
chromium metal may be electrolytically de-  
posited directly upon iron, steel or other fer-  
rous metal (such as predominantly ferrous  
alloy steels) provided the ferrous metal is  
35 preliminarily subjected to a suitable heat-  
treatment, followed by an adequate clean-  
ing of its surface.

Following is a preferred method of carry-  
ing out the invention, which is not however  
40 limited to the particular manipulations and  
operating conditions recited by way of ex-  
ample:

The ferrous article to be plated, for ex-  
ample in the form of a sheet or if desired of  
45 a fashioned implement or article, is first  
heated to dull redness, and permitted to cool,  
preferably slowly. The surfaces are then  
thoroughly cleaned by suitable chemical or  
mechanical methods or combinations of  
50 these. The cleaning method which I now

prefer is as follows, although it forms no  
part of the present invention:

The heat-treated article is immersed in a  
hot solution of hydrochloric acid, for ex-  
55 ample 20% HCl at 85° C., until all oxid is  
removed, after which it is immersed in a  
hot solution of caustic soda. The article  
is then connected as the cathode in a 10%  
solution of sulfuric acid and subjected to a  
60 high current density, say 150 amperes per  
square foot for five minutes. It is immedi-  
ately transferred to a suitable chromi-  
plating bath and plated under standard con-  
ditions. I prefer to employ a bath consist-  
65 ing of an aqueous solution of chromic acid  
containing a relatively small proportion of  
chromic sulfate, although any other suitable  
plating solution may be used.

Articles prepared as above will be found  
quite free from pin holes and like defects,  
70 even when the chromium coating is extreme-  
ly thin, or of the "flash" type. Naturally,  
the perfection of the coating is dependent  
upon the care with which the several oper-  
ations are carried out; and with sufficient  
75 care coatings which are absolutely continu-  
ous may be applied over large areas. So  
far as I am aware, such continuous or prac-  
tically continuous coatings of chromium  
have not heretofore been secured directly  
80 upon ferrous metal surfaces.

I claim:

1. In the art of electrodepositing chro-  
mium on iron, steel and predominantly fer-  
rous alloys, that improvement which com-  
85 prises heating the aforesaid material of fer-  
rous character to a dull redness, thereupon  
cooling the heated material, and immediate-  
ly cleaning the surface of the cool material.

2. In the art of electrodepositing chro-  
mium on iron, steel and predominantly fer-  
rous alloys that improvement, which com-  
90 prises heating the material of ferrous char-  
acter to a dull redness, slowly cooling the  
heated material, immediately cleaning the  
95 cool material with warm dilute hydrochloric  
acid until the surface film on said material is  
removed, then subjecting said material to the  
action of hot caustic soda solution and finally  
100 electrolytically cleaning the thus treated ma-

terial in a dilute sulphuric acid medium under the action of an electric current of a character sufficient to give a high current density.

3. The method of electrodepositing continuous platings of chromium on iron, steel and predominantly ferrous alloys, which comprises heating the aforesaid material of ferrous character to a dull redness, thereupon cooling the heated material, and immediately electrodepositing chromium on the freshly cleaned surface of the material whereby a practically continuous plating of chromium is made on the material.

4. The method of electrodepositing continuous platings of chromium on iron, steel and predominantly ferrous alloys, which comprises heating the material of ferrous character to a dull redness, slowly cooling the heated material, immediately cleaning the cool material with warm dilute hydrochloric acid until the surface film on said material is removed, then subjecting said material to the action of hot caustic soda solution, finally electrolytically cleaning the thus treated material in a dilute sulphuric acid medium under the action of an electric current of a character sufficient to give a high current density and immediately thereafter electrodepositing chromium on the freshly cleaned surface of the material whereby a practically continuous plating of chromium is made on the material.

In testimony whereof, I affix my signature.  
VINCENT M. VERTUCCI.

35

40

45

50

55

60

65